

FIP 8309

XR 1,633,213

Patented June 21, 1927.

1,633,213

## UNITED STATES PATENT OFFICE.

JOSEPH FRANCIS KING, OF BROOKLYN, NEW YORK, ASSIGNOR TO HERMAN A. METZ,  
OF NEW YORK, N. Y.

## CHEMICAL COMPOSITION.

No Drawing.

Application filed January 19, 1926. Serial No. 82,348.

This invention relates to a product and process for cleaning, whitening, filling and weighting fabric materials.

In the usual methods now employed for weighting, filling, cleaning and whitening gray materials, it is necessary to preliminarily bleach the materials with chlorine gas or peroxide which acts upon the iron tanks and causes rust stains, so that in the separate and distinct further steps of the process and treatment of the goods, these stains will be maintained so that when the goods are dyed, weighted and filled in succeeding operations, they will materially affect the quality of the goods. Furthermore where the steps are carried out separately without sufficient active ingredients to cause the weighting and filling materials to enter the fibers, the weighting materials will be merely disposed upon the surface and therefore readily removed during subsequent washing.

An object of the invention is the provision of a product adapted to be placed in solution for use in a wood or iron kier for thoroughly removing foreign matter, and for whitening, filling and weighting such materials as rayon, cotton, wool, silk, linen and other plant or fibrous materials.

A further object of the invention is the provision of a process in which the fabric materials are cleaned, whitened, weighted and filled in a single operation with ingredients which will not cause rust stains, but which will thoroughly impregnate the fiber so that the filling and weighting materials are thoroughly embedded, and therefore will not be readily removed for subsequent washing.

This invention will be best understood from a consideration of the following detailed description forming a part of the specification; nevertheless it is to be understood that the invention is not confined to the disclosure, being susceptible of such changes and modifications which shall define no material departure from the salient features of the invention as expressed in the appended claims.

In carrying out my process, I employ the following ingredients in approximately the proportions noted, for producing five-hundred (500) pounds of the materials:

300 pounds sodium perborate.

50 pounds cornstarch (pure white).

55 30 pounds sodium tripolyphosphate (crystals).

25 pounds aluminum sulphate powder (free of iron).

75 pounds Epsom salts (crystals).

20 pounds denatured alcohol.

In this composition are included certain ingredients or agents which are used as detergents for freeing the materials of resinous matters and impurities such as specks, shives and motes, and for filling and weighting. The filling and weighting material such as cornstarch, denatured alcohol and Epsom salts may be omitted entirely or in part when the materials to be treated are required to be of a softer texture, and in such a case the quantity of sodium tripolyphosphate is increased. When the weighting and filling materials are to be omitted, the remaining ingredients are used in the following proportions:

300 pounds sodium perborate.

125 pounds sodium tripolyphosphate (crystals).

50 pounds Epsom salts (crystals).

25 pounds aluminum sulphate powder (free of iron).

As an example of the treatment for one-hundred (100) pounds of the materials of standard base, three to four per cent of the first mentioned composition is dissolved into a ninety-six to ninety-seven percent of water solution.

The materials having been placed in the tank, cold water is run through the tank in the usual manner and then the previously dissolved solution is forced into the tank after the cold water has been drained off, and the solution with the goods is boiled from four to six hours under a pressure.

It has been the practice to fill, weight, and size rayon and other cotton materials in the final treatment so that the materials are given a fugitive or false weight since the ingredients are merely deposited on the surface of the material and not into the fibers so that the usual artificial finishing is lost.

By my particular method of placing all of the ingredients and of the particular type in the kier solution and in boiling them from four to six hours, goods of a superior quality is had, and in which the fibers of the materials are impregnated with the weighting and filling ingredients, and it is unnecessary by this method to give any previous treatments, the thorough impregnation of the materials being due to the high

penetrating power of the ingredients used in the kier solution.

While I have given certain proportions of the ingredients to be used, it must be borne

5 in mind that these proportions are merely approximate, and may be varied without materially affecting the efficiency of the solution.

I claim:—

10 1. A composition of the character described, comprising 300 pounds sodium perborate, 50 pounds cornstarch, 30 pounds sodium triphosphate, 25 pounds aluminum sulphate powder, 75 pounds Epsom salts, and 20 pounds denatured alcohol.

15 2. A composition of the character de-

scribed, comprising 12 parts by weight of sodium perborate, 1.2 parts sodium triphosphate, 3 parts Epsom salts and 1 part of aluminum sulphate powder.

20 3. A process for making a cleaning, filling, and weighting solution which comprises mixing 300 pounds sodium perborate, 50 pounds cornstarch, 30 pounds sodium triphosphate, 25 pounds aluminum sulphate 25 powder, and 75 pounds Epsom salts and 20 pounds denatured alcohol, dissolving in water a quantity of the materials which represent from 3 to 4% of the weight of the material to be treated.

JOSEPH FRANCIS KING.